

## UNITED STATES PATENT OFFICE.

ALBERT A. SOMERVILLE, OF FLUSHING, NEW YORK, ASSIGNOR OF TWO-THIRDS TO  
R. T. VANDERBILT COMPANY, INCORPORATED, OF NEW YORK, N. Y., A CORPORA-  
TION OF NEW YORK.

## OIL COMPOSITION.

No Drawing.

Application filed June 19, 1926. Serial No. 117,203.

This invention relates to improvements in petroleum oil compositions. More particularly, the invention includes improved petroleum oil compositions suitable for use at high 5 temperatures or under exposure to the air, and having improved stability when so used. The new petroleum oil compositions are valuable for use for lubricating purposes both at ordinary and at high temperatures, as well 10 as for use in transformers or oil switches, in cable impregnation, or for other electrical purposes.

When mineral oil lubricants are used in internal combustion engines, the high temperature to which the oils are subjected results in more or less rapid deterioration with 15 loss of lubricating properties, particularly where air comes in contact with the oils at the same time that they are subjected to heat 20 and the oils undergo more or less decomposition, with the attendant formation of carbon or sludge-like ingredients. So also when lubricating oils are used under air pressures as in air compressors, a great deal of trouble 25 is often experienced due to the lubricating oil gumming after a few days' use. Similarly, when hydrocarbon oils are used in transformers or for cable impregnation, where the oil is subjected to an elevated tem- 30 perature for prolonged periods of time, it undergoes or tends to undergo deterioration, particularly in its electrical properties, so that the oil would have to be removed and replaced at more or less frequent intervals, 35 e. g., in transformers or in the saturating bath used for impregnating the wrappings of cables.

The present invention provides an improved oil composition which can be used for 40 prolonged periods of time as compared with ordinary oil compositions, and which is stabilized so that it will resist deterioration during use at high temperatures. The improved oil compositions can also be used at 45 lower temperatures where they are subjected during use to oxidation, with resulting ten- 50 dency toward deterioration, as where subjected to air pressure in air compressors, etc.

According to the present invention, the lubricating oil or transformer oil or cable impregnating oil or grease, etc., has compounded therewith a small amount of a condensation product of a ketone with a nitrogenous base, which condensation product 55 serves as a stabilizing agent to retard or pre-

vent deterioration at high temperatures or under oxidizing conditions at lower tem- 60 perature.

In the case of lubricating oil compositions, the lubricating oil may be the same as or 65 similar to lubricating oils now commonly used at high temperatures, such as in gas engines and internal combustion engines, or such as are used at lower temperatures un- 70 der air pressure as in air compressors. The 65 oils may vary from light lubricating oils to heavier lubricating oils. In general, these oil's are hydrocarbon oils, although they may have small amounts of vegetable or animal 75 oils compounded therewith.

In the case of transformer oils or cable 80 saturating oils or greases, the oil or grease may be of the kind commonly used for such purposes with the stabilizing agent added thereto.

The stabilizing materials, which are added 85 in small amounts to the oils or oil compositions, are condensation products of ketones with nitrogenous bases, such as ammonia and amines. In general, the compounds 90 added should be non-volatile at the tempera- 85 ture at which the lubricating oil is to be used, and should also be stable in the sense that they are not decomposed into volatile or objectionable compounds at the tempera- 95 ture of use. The material should also be soluble in the oil to such an extent that it will form a homogeneous admixture there- 100 with.

The stabilizing ingredients or ingredient 90 may be added directly to the oil, if readily soluble therein, or the dissolving of the sta- 105 bilizing material may be promoted by heating, or the material may be first dissolved in a solvent such as benzol, and the benzol solu- 95 tion then added to the oil, with subsequent heating of the composition to drive off the benzol.

The amount of the stabilizing material 100 which it is necessary to add is small. In general, a few per cent at most will suffice, and as little of a fraction of a per cent may be sufficient, e. g., 0.5% to 1%.

The invention will be further illustrated 105 by the following specific examples, but it is intended and will be understood that the invention is illustrated thereby but is not limited thereto.

A lubricating oil composition such as is 110 commonly used for the lubrication of auto-

mobile engines has added thereto a small amount, e. g., 0.5% to 1% of a condensation product of acetone with ammonia, the admixture being promoted by dissolving the condensation product in benzol and then intimately admixing the benzol solution with the lubrication oil and subsequently distilling off the benzol. The resulting lubricating oil composition will have improved stability and resistance to decomposition at the elevated temperatures at which it is used in automobile and similar internal combustion engines.

In a similar manner, a mineral oil composition such as commonly used for impregnating the paper wrappings of cables may have a similar amount of the same condensation product added thereto in a similar manner. When the resulting composition is used for saturating the paper wrapping of cables, by passing the cable through the hot saturating bath, the bath will retain high insulating properties for long periods of time. In fact, the bath may be increased in its electrical resistivity over that of the original oil, being in this respect radically different from the ordinary saturating bath which rapidly deteriorates in its electrical resistivity.

In a similar manner, oils such as are used for transformers, or for electrical switches, etc., can be similarly treated with a small amount of the condensation product.

Among the condensation products of ketones with nitrogenous bases which may be particularly mentioned, are condensation products of ammonia with acetone. The action of ammonia on acetone results in the formation of a mixture of acetone amines, such as diacetone amine, triacetone amine, etc. This condensation of ammonia with acetone can be facilitated by using a dehydrating agent such as calcium chloride, etc. A suitable method of making the condensation product is to introduce ammonia gas into acetone containing powdered calcium chloride in suspension until the acetone is saturated, and then allowing the reaction mixture to stand until the reaction is completed. The resulting oily product can be freed from excess acetone and ammonia by

distillation and can be further treated to separate the different acetone amine products or fractions therefrom. Instead of using acetone, other ketones can be employed, and instead of using ammonia, certain amines, for example, hydroxyl amine.

The action of the condensation product as a stabilizing agent is somewhat obscure, but apparently it is due to prevention of oxidation at the elevated temperatures to which the oil compositions are subjected in use, and particularly where air or oxygen comes into contact with the oil, although the stabilizing ingredients are used only in small amounts, not usually exceeding about 2%, and in some cases being only a fraction of a per cent. Nevertheless, they impart improved stability to the oil compositions at elevated temperatures.

I claim:

1. An improved petroleum oil composition comprising petroleum oil having combined therewith a small amount of a condensation product of a ketone with a nitrogenous base.
2. A cable impregnating oil composition comprising a mineral oil or grease adapted for use for cable impregnation having combined therewith a small amount of a condensation product of a ketone with a nitrogenous base.
3. An improved petroleum oil composition comprising petroleum oil having combined therewith a small amount of a condensation product of a ketone with ammonia.
4. A cable impregnating oil composition comprising a mineral oil or grease adapted for use for cable impregnation having combined therewith a small amount of a condensation product of a ketone with ammonia.
5. An improved petroleum oil composition comprising petroleum oil having combined therewith a small amount of a condensation product of acetone with ammonia.
6. A cable impregnating oil composition comprising a mineral oil or grease adapted for use for cable impregnation having combined therewith a small amount of a condensation product of acetone with ammonia.

In testimony whereof I affix my signature.

ALBERT A. SOMERVILLE.